

## UNITED STATES PATENT OFFICE

2,432,456

FROTH FLOTATION OF A NICKEL-COPPER  
SULFIDE MATTE

William Kelvin Sproule, George Alan Harcourt,  
and Ernest Herbert Rose, Copper Cliff, Ontario,  
Canada, assignors to The International Nickel  
Company, Inc., New York, N. Y., a corporation  
of Delaware

No Drawing. Application September 19, 1945,  
Serial No. 617,450. In Canada March 14, 1945

16 Claims. (CL 241-20)

1

The present invention relates to a novel flotation process for concentrating comminuted matte consisting principally of nickel sulfide, copper sulfide, and a metallic copper-nickel alloy into a copper concentrate substantially free from nickel sulfide and a nickel concentrate substantially free from copper sulfide and to a flotation reagent therefor.

Heretofore, many flotation reagents have been proposed for the selective flotation of copper sulfide minerals from copper ores. Although attempts have been made to discover the chemical properties which result in a substance acting as a good collecting agent, no general principles have been established which will enable a person skilled in the art to predict with certainty whether or not a reagent will have superior collecting properties for copper sulfide minerals. Similarly, one skilled in the art cannot predict whether or not a compound will give satisfactory results in the segregation of copper sulfide and nickel sulfide from a matte consisting principally of copper sulfide, nickel sulfide and a metallic copper-nickel alloy. While it has been stated that the presence of trivalent nitrogen or divalent sulfur causes a compound to be a good collector for copper sulfide minerals, nevertheless substances such as triphenyl guanidine, mercapto-benzothiazol and the product of the reaction between butyl amine and n-valeraldehyde, all of which contain trivalent nitrogen or divalent sulfur, do not in all cases afford satisfactory separation of copper sulfide from nickel sulfide.

It is, of course, true that many empirically discovered collecting reagents for copper sulfide minerals have been patented. For example, in U. S. Patent No. 1,364,308, Perkins et al. propose the use of aromatic thiourea compounds such as thiocarbanilide or diphenyl thiourea for the flotation of ores, such as the Utah Copper Company's ore consisting principally of chalcocite, chalcopyrite and gangue. These patentees state that pine oil should be added to obtain good frothing qualities. In U. S. Patent No. 2,180,926, Jayne discloses the use of substituted biguanides, their salts and aldehyde condensation products in the selective flotation of copper sulfide minerals from ore containing chalcocite, bornite, enargite and pyrite. In U. S. Patent No. 1,610,217, Elley discloses the flotation of Phelps-Dodge Corporation Copper Queen ore by the use of alkyl-substituted thioureas such as dibutylthiourea.

In our process, a flotation reagent is desired which has so high a preference for copper sulfide that a considerably greater percentage of copper

2

sulfide is caused to float than is the case with the reagents proposed by the prior art and particularly by the above-mentioned patentees. In addition, these results must be obtained with a matte or raw material comprising substantially all copper sulfide, nickel sulfide and a metallic copper-nickel alloy, that is to say, a matte substantially free from iron. Thus, the novel collecting reagents for our process give unusually good results when used with a matte or raw material consisting principally of copper sulfide, nickel sulfide and a metallic copper-nickel alloy but do not give commercially satisfactory results when used with an unsmelted ground Sudbury ore containing a considerable amount of iron and consisting of pyrrhotite, chalcopyrite, pentlandite and gangue.

It is an object of the present invention to employ a novel flotation agent for our process which is capable of yielding greatly improved results in the separation of copper sulfide and nickel sulfide from mattes or raw materials consisting principally of copper sulfide, nickel sulfide and a metallic copper-nickel alloy, and which is capable of being utilized in a practical manner on an industrial scale with conventional flotation equipment.

The present invention also contemplates the utilization of a flotation process on comminuted matte or raw material consisting principally of copper sulfide, nickel sulfide and a metallic copper-nickel alloy having as end products nickel sulfide substantially free from copper sulfide and copper sulfide substantially free from nickel sulfide.

It is within the scope of the present invention to employ a novel flotation reagent for our process which will float copper sulfide as a froth recoverable as a copper-rich concentrate and which will cause nickel sulfide to be depressed, whence it may be recovered as a nickel-rich concentrate.

It is a feature of the present invention that outstanding results are obtained without necessarily using an auxiliary frothing agent and within a much shorter time of flotation as compared with the flotation reagents of the prior art.

Various other objects, advantages and features of the present invention will become apparent from the following detailed description.

We have discovered that diphenyl guanidine and diortho tolyl guanidine, when used as flotation reagents, effect outstanding separation of nickel sulfide and copper sulfide from mattes consisting principally of nickel sulfide, copper sulfide and a metallic copper-nickel alloy.

The matte is preferably prepared for the flotation operation as described in our co-pending applications Serial No. 527,510, now U. S. Patent No. 2,419,973, and Serial No. 527,511. Although this process can be applied to mattes containing about 8% to about 30% or more sulfur and the balance substantially all copper and nickel in any proportions, the preferred matte compositions are about 30% to 65% nickel, 20% to 24% sulfur and 50% to 15% copper. It will be understood by those skilled in the art that this preferred range of compositions applies particularly to ore which has been treated in a blast furnace or reverberatory furnace and then blown to bessemer matte. However, matte or raw material having the above-noted composition may be obtained by melting together scrap copper-nickel alloys and sulfur in the desired proportions or in any other suitable manner.

As the matte leaves the bessemer converter it is in the molten state. If the matte is not molten, it is heated until fusion occurs. The molten matte is slowly cooled from the temperature at which crystallization begins to a temperature of about 950° F. or lower, the cooling occurring over a period of about 1 day to about 15 days. However, more satisfactory results are obtained if the slow cooling is continued to a temperature of about 200° F. We have found that the slow cooling is particularly important within the temperature range of about 1300° F. to about 950° F. The slowly cooled matte consists of mechanically joined crystals of nickel sulfide, copper sulfide and copper-nickel alloy, these crystals being of sufficient size that they may be mechanically separated, for example, by crushing and grinding. Although we have described, in detail, a method of preparing material suitable for use with our novel flotation process, it is to be understood that we do not limit ourselves to this particular method of preparation.

According to the invention, the slowly cooled matte is crushed and ground to such a degree of fineness that the crystals of nickel sulfide, copper sulfide and copper-nickel alloy are substantially freed from each other and are capable of being treated by flotation. We prefer to grind the matte until all the material will pass a 100-mesh screen and about 5% to about 50% is retained on a 325-mesh screen. Sufficient water is added to the matte during grinding to form a pulp whose solid content is between about 10% and about 40%. A sufficient amount of a suitable alkaline reagent, for example lime, is added to maintain a pH of about 12.4. This pH value is not critical however and, broadly speaking, may vary within the ranges of about pH 10.0 to about pH 12.4 when using lime. Of course, certain other alkaline reagents such as sodium hydroxide may be utilized, but we have found the use of lime preferable.

We also add between about 0.25 pound and 1.0 pound of our novel flotation reagent, to wit: diphenyl guanidine or diortho tolyl guanidine, per ton of matte, at the grinding mill. The pulp is then treated by froth flotation. Sufficient froth is commonly produced without the aid of any auxiliary frothing agents. However, if additional frothing is desired, a suitable auxiliary frothing agent, such as pine oil, may be added. The copper sulfide is floated and may be drawn off with the froth as a copper concentrate containing only about 1% to about 10% nickel sulfide. The nickel sulfide together with the larger portion of the metallics is depressed and is withdrawn as a nickel

concentrate containing only about 0.5% to about 5% copper sulfide.

In commercial practice, it has been found advantageous to carry out the flotation operation in a series of three to six roughing and cleaning stages and to regrind the copper rougher concentrate, and sometimes the nickel concentrate, before cleaning. Magnetic material consisting largely of copper-nickel alloy is removed from the pulp either before flotation, or from the flotation products or at both stages of the process. This magnetic material may be treated by known methods. After nickel and copper concentrates of desired purity are obtained, they are each de-watered and marketed or treated in any suitable manner to recover metallic nickel and metallic copper from the sulfides.

For a better understanding of the present invention by those skilled in the art, the following specific and illustrative examples are given:

*Example No. 1*

A typical bessemer matte having the following composition was used:

|    | Element                     | Per cent |
|----|-----------------------------|----------|
| 25 | Nickel                      | 40.4     |
|    | Copper                      | 37.0     |
|    | Sulfur                      | 21.8     |
| 30 | Iron                        | .57      |
|    | Silica and other impurities | 23       |
|    | Total                       | 100.00   |

The matte, which was at a temperature of about 35 1600° F. and still molten from its production, was slowly cooled to a temperature of about 300° F. over a period of about 16 days. The cooled, solidified matte was crushed and then ground in a saturated aqueous solution of hydrated lime to which about 0.5 pound of diphenyl guanidine was added per ton of matte. The grinding was continued until all the material would pass through a 100-mesh screen and about 35% was retained on a 325-mesh screen.

40 The finely ground matte was found to consist of discrete, mechanically freed particles of copper sulfide, nickel sulfide and a metallic copper-nickel alloy which, together with the hydrated lime and diphenyl guanidine, formed a pulp having a pH of about 12.4 and a pulp density of about 25% solids. After being discharged from the grinding mill, the pulp was introduced into a mechanical type flotation cell. Due to the novel collecting action of the diphenyl guanidine, the copper sulfide together with a small portion of the metallics was selectively floated and concentrated into the froth to form a rougher copper concentrate while the nickel sulfide together with the remainder of the metallics was depressed to 55 form a rougher nickel concentrate. It was not necessary to add a further frothing agent to the pulp as sufficient frothing resulted from the use of the diphenyl guanidine.

In this manner, the copper sulfide was to a 60 large extent separated from the nickel sulfide. However, the rougher copper concentrate still contained about 14.5% nickel and, accordingly, further purification was desirable. To this end, the rougher copper concentrate was regrind 65 ed in the presence of about 0.4 pound of diphenyl guanidine per ton of matte together with sufficient hydrated lime to maintain a pH of about 12.4. The grinding was continued until all the material would pass through a 200-mesh screen and about 7% was retained on a 325-mesh

screen. The resulting pulp, having a density of about 15% solids, was floated and, as previously described, separated into a froth containing copper sulfide together with a small portion of the metallics and into a depressed nickel concentrate containing nickel sulfide together with the remainder of the metallics. The cleaned copper concentrate containing about 62.0% copper and about 6.5% nickel was subjected, without further grinding to a third flotation operation, the pulp density being about 12% solids. The re-cleaned copper concentrate was dewatered and passed through a magnetic separator, thus being divided into a magnetic portion consisting mostly of nickel-copper alloy and a final copper product consisting of substantially pure copper sulfide having a low nickel content of about 4.5%.

The nickel sulfide product from the recleaning operation was combined with the nickel products of the two previous flotation steps. The resulting nickel concentrate was passed through a magnetic separator which formed a magnetic product consisting largely of copper-nickel alloy and a non-magnetic final nickel concentrate. These results were obtained in the unusually short total floating time of 18 minutes. The final dried products obtained had the following assays and represented the following recoveries:

| Material       | Assay       |             | Recovery    |             |
|----------------|-------------|-------------|-------------|-------------|
|                | Per cent Cu | Per cent Ni | Per cent Cu | Per cent Ni |
| Feed           | 37.0        | 40.4        | 100.00      | 100.0       |
| Cu Concentrate | 75.0        | 4.5         | 83.2        | 4.6         |
| NI Concentrate | 1.4         | 67.3        | 1.4         | 61.8        |
| Metallics      | 26.0        | 82.0        | 15.4        | 33.6        |

#### Example No. 2

A typical bessemer matte having the following composition was used:

| Element                     | Per cent |
|-----------------------------|----------|
| Nickel                      | 52.5     |
| Copper                      | 24.5     |
| Sulfur                      | 22.3     |
| Iron                        | .50      |
| Silica and other impurities | .20      |
| Total                       | 100.00   |

Eighteen tons of this matte, still molten from its production, were slowly cooled from 2100° F. to a temperature of 370 F. over a period of 8 days. A portion of the cooled, solidified matte was treated and subjected to a flotation operation in a manner similar to that described in connection with Example No. 1. The final products obtained after recleaning and magnetic separation had the following assays and represented the following recoveries:

| Material       | Assay       |             | Recovery    |             |
|----------------|-------------|-------------|-------------|-------------|
|                | Per cent Cu | Per cent Ni | Per cent Cu | Per cent Ni |
| Feed           | 24.5        | 52.5        | 100         | 100         |
| Cu Concentrate | 76.0        | 2.9         | 69.9        | 1.3         |
| NI Concentrate | 1.52        | 70.0        | 3.3         | 70.0        |
| Metallics      | 26.0        | 59.9        | 26.3        | 28.7        |

It is to be understood that the preceding examples are purely illustrative of our invention and that many changes can be made therein by one skilled in the art without departing from

the spirit and scope of the invention. For example, although with the particular matte compositions illustrated a metallic copper-nickel alloy appeared in the slowly cooled matte, it is apparent that no metallics will be formed if the sulfur present in the original charge is sufficient to combine with all the copper and nickel present. In this case the magnetic separation step could be dispensed with and the final products of the flotation process would be substantially pure copper sulfide and substantially pure nickel sulfide, both of these compounds being free from metallics.

It is also within the purview of the invention to magnetically separate the metallic copper-nickel alloy from the sulfides before flotation.

Moreover, those skilled in the art will recognize that the amount of each reagent required to produce a clean concentrate by froth flotation cannot be stated precisely. It is well recognized by those skilled in the art that, as in the case of naturally occurring ores, different samples of matte of similar composition will require slightly different amounts of the various reagents. Accordingly, those skilled in the art will recognize that the various amounts of reagents set forth hereinbefore are purely illustrative of the general magnitude of the quantities involved and that variations will occur dependent upon various local conditions.

Furthermore, while the present process has been described in conjunction with bessemer matte produced from Sudbury ore, it is to be understood that the present process can be utilized with equally satisfactory results in the separation of metallic nickel from metallic copper. In such an application of the present process, copper-nickel scrap, for example, can be melted with sufficient sulfur to provide a product having essentially the same composition as bessemer matte and this synthetic bessemer matte can then be subjected to regulated slow cooling in the same manner as bessemer matte produced in the treatment of Sudbury or other copper-nickel sulfide ores. Similarly, other materials containing copper and nickel, but devoid of or containing only small amounts of sulfur, can be sulfidized to produce a matte consisting essentially of copper, nickel and sulfur and the matte so produced subjected to regulated slow cooling followed by comminution and separation of the comminuted material into a product consisting essentially of copper sulfide and a product consisting essentially of nickel sulfide. In this connection, it is to be noted that in the separation of the comminuted crystallized sulfides in accordance with the preferred embodiment of the present invention both the nickel-rich fraction and the copper-rich fraction are termed concentrates although the material of the nickel concentrate is depressed while the material of the copper concentrate is floated and removed in the froth.

We claim:

1. A process for recovering copper sulfide and nickel sulfide from bessemer matte essentially devoid of iron which comprises slowly cooling said bessemer matte from the molten state to a temperature below about 950° F. to form a mass containing mechanically joined crystals of copper sulfide and nickel sulfide together with a copper-nickel alloy, comminuting the slowly-cooled mass in the presence of a sufficient quantity of an alkaline reagent to maintain a pH of about 10.0 to about 12.4, adding about 0.25 to about 1.0 pound of a compound selected from the group

consisting of diphenyl guanidine and diortho tolyl guanidine per ton of matte, subjecting the comminuted mass to froth flotation whereby copper sulfide is floated and recovered in the froth as a copper concentrate, the nickel sulfide being depressed as a nickel concentrate, and removing said copper-nickel alloy from said copper concentrate and said nickel concentrate by magnetic separation.

2. A process for separating nickel sulfide and copper sulfide as concentrates from a ground, slowly-cooled bessemer matte substantially free from iron and containing an appreciable quantity of a copper-nickel alloy which comprises subjecting said ground, slowly-cooled matte to froth flotation at a pH of about 10.0 to about 12.4 in the presence of about 0.25 to about 1.00 pound of a compound selected from the group consisting of diphenyl guanidine and diortho tolyl guanidine per ton of matte to form a depressed rougher nickel concentrate and a floated rougher copper concentrate, treating said rougher copper concentrate by selective froth flotation to obtain a purified copper concentrate together with an additional quantity of nickel concentrate, and removing said copper-nickel alloy from said copper concentrate by magnetic separation.

3. A process for recovering copper sulfide and nickel sulfide from bessemer matte which comprises slowly cooling said bessemer matte from the molten state to a temperature below about 950° F. to form a mass containing copper sulfide, nickel sulfide and a copper-nickel alloy, comminuting the slowly-cooled mass in the presence of a sufficient quantity of an alkaline reagent to maintain a pH of about 10.0 to about 12.4 and a pulp density of about 25% solids, adding about 0.25 to about 1.0 pound of diphenyl guanidine per ton of matte, subjecting the comminuted mass to froth flotation whereby copper sulfide is floated and recovered in the froth as a copper concentrate, the nickel sulfide being depressed as a nickel concentrate, and removing at least a portion of said copper-nickel alloy by magnetic separation.

4. A process for separating nickel sulfide and copper sulfide as concentrates from a ground, slowly-cooled bessemer matte substantially free from iron and containing an appreciable quantity of a copper-nickel alloy which comprises subjecting said ground, slowly-cooled matte to froth flotation while maintaining a pH of about 10 to about 12.4 in the presence of a compound selected from the group consisting of diphenyl guanidine and diortho tolyl guanidine to form a depressed rougher nickel concentrate and a floated rougher copper concentrate, treating said rougher copper concentrate by selective flotation to obtain a purified copper concentrate together with an additional quantity of nickel concentrate, and removing said copper-nickel alloy from said copper concentrate and said nickel concentrate by magnetic separation.

5. A process for separating and recovering nickel sulfide and copper sulfide as concentrates from a smelted mass substantially free from iron and containing mechanically joined crystals of nickel sulfide and copper sulfide which comprises comminuting said mass to a size finer than 100-mesh in a saturated aqueous solution of hydrated lime to obtain a pH of about 12.4 and a pulp density between about 10% and about 40% solids, adding about 0.5 pound of diphenyl guanidine per ton of mass while grinding, treating the comminuted mass by froth flotation whereby the copper sulfide is floated as a copper concentrate

and the nickel sulfide is depressed as a nickel concentrate, and further purifying the copper concentrate by successive froth flotation steps in the presence of diphenyl guanidine.

6. A process for separating and recovering nickel sulfide and copper sulfide as concentrates from a smelted mass essentially free from iron and containing mechanically joined crystals of nickel sulfide and copper sulfide which comprises 10 comminuting said mass in a saturated aqueous solution of hydrated lime until about 35% thereof is retained on a 325-mesh screen, adding about 0.5 pound of diphenyl guanidine per ton of mass while grinding, treating the comminuted mass by froth flotation while maintaining a pH of about 10.0 to about 12.4 whereby the copper sulfide is floated as a copper concentrate and the nickel sulfide is depressed as a nickel concentrate, and further purifying the copper concentrate by successive froth flotation steps in the presence of about 0.5 pound of diphenyl guanidine per ton.

7. A process for recovering copper sulfide and nickel sulfide from bessemer matte substantially free from iron which comprises slowly cooling 25 said bessemer matte from the molten state to a temperature below about 950° F. over a period of about one to about fifteen days, comminuting the slowly-cooled matte to a size finer than about 100-mesh in the presence of a sufficient quantity 30 of an alkaline reagent to maintain a pH of about 10.0 to about 12.4, adding about 0.25 to about 1.0 pound of diphenyl guanidine per ton of mass, and subjecting the comminuted mass to froth flotation whereby copper sulfide is floated and 35 recovered in the froth as a copper concentrate, the nickel sulfide being depressed as a nickel concentrate.

8. A process for separating nickel sulfide and copper sulfide as concentrates from a ground, 40 slowly-cooled bessemer matte which comprises subjecting said ground, slowly-cooled matte to froth flotation while maintaining a pH of about 10 to about 12.4 in the presence of a compound selected from the group consisting of diphenyl 45 guanidine and diortho tolyl guanidine to form a depressed rougher nickel concentrate and a floated rougher copper concentrate, and treating said rougher copper concentrate by selective froth flotation to obtain a purified copper concentrate 50 together with an additional quantity of nickel concentrate.

9. A process for separating nickel sulfide and copper sulfide as concentrates from a ground, slowly-cooled bessemer matte which comprises 55 subjecting said ground, slowly-cooled matte to froth flotation while maintaining a pH of about 10 to about 12.4 in the presence of about 0.25 to about 1.00 pound of a compound selected from the group consisting of diphenyl guanidine and diortho tolyl guanidine per ton of matte to form 60 a depressed rougher nickel concentrate and a floated rougher copper concentrate, and treating said rougher copper concentrate by selective froth flotation to obtain a purified copper concentrate 65 together with an additional quantity of nickel concentrate.

10. A process for separating and recovering nickel sulfide and copper sulfide as concentrates from a smelted mass substantially devoid of iron 70 and containing mechanically joined crystals of nickel sulfide and copper sulfide which comprises comminuting said mass in a saturated aqueous solution of hydrated lime, adding about 0.25 to about 1.00 pound of diphenyl guanidine per ton 75 of matte while grinding, subjecting the ground

mass to froth flotation while maintaining a pH of about 10.0 to about 12.4 whereby the copper sulfide is floated as a copper concentrate and the nickel sulfide is depressed as a nickel concentrate, and further purifying the copper concentrate by successive froth flotation steps in the presence of diphenyl guanidine.

11. A process for recovering copper sulfide and nickel sulfide from bessemer matte which comprises slowly cooling said bessemer matte from the molten state to a temperature below about 950° F., comminuting the slowly-cooled matte in the presence of a sufficient quantity of an alkaline reagent to maintain a pH of about 10.0 to about 12.4, adding about 0.25 to about 1.0 pound of a compound selected from the group consisting of diphenyl guanidine and diortho tolyl guanidine per ton of matte, and subjecting the comminuted mass to froth flotation whereby copper sulfide is floated and recovered in the froth as a copper concentrate, the nickel sulfide being depressed as a nickel concentrate.

12. A process for separating nickel sulfide from copper sulfide which comprises subjecting a comminuted copper-nickel matte substantially devoid of iron and containing discrete particles of nickel sulfide and copper sulfide to selective froth flotation after adding about 0.25 to about 1.00 pound of a compound selected from the group consisting of diphenyl guanidine and diortho tolyl guanidine per ton of matte while maintaining a pH of about 10.0 to about 12.4 whereby the copper sulfide is floated for recovery in the froth and the nickel sulfide is depressed.

13. A process for separating nickel sulfide from copper sulfide which comprises subjecting a comminuted smelted mass substantially devoid of iron and containing discrete particles of nickel sulfide and copper sulfide to selective froth flotation after adding a compound selected from the group consisting of diphenyl guanidine and diortho tolyl guanidine while maintaining a pH of about 10 to about 12.4 and a pulp density between about 10% and about 40% solids whereby the copper sulfide is floated for recovery in the froth and the nickel sulfide is depressed.

14. A process for separating and recovering nickel sulfide and copper sulfide as concentrates from a bessemer matte containing mechanically joined crystals of nickel sulfide and copper sulfide which comprises comminuting said matte in a saturated aqueous solution of hydrated lime, adding about 0.25 to about 1.00 pound of diphenyl guanidine per ton of matte while grinding, subjecting the comminuted matte to froth flotation whereby the copper sulfide is floated as a copper concentrate and the nickel sulfide is depressed as a nickel concentrate, further purifying the copper concentrate by successive froth flotation steps in the presence of diphenyl guanidine, and combining the nickel concentrates from said froth flotation steps.

15. A process for separating nickel sulfide from copper sulfide which comprises subjecting a comminuted smelted mass substantially devoid of iron and containing discrete particles of nickel sulfide and copper sulfide to selective froth flotation while maintaining a pH of about 10 to about 12.4 after having added diphenyl guanidine whereby the copper sulfide is floated for recovery as a froth and the nickel sulfide is depressed.

16. A process for separating nickel sulfide from copper sulfide which comprises subjecting a comminuted bessemer matte containing discrete particles of nickel sulfide and copper sulfide to selective froth flotation while maintaining a pH of about 10 to about 12.4 after adding a compound selected from the group consisting of diphenyl guanidine and diortho tolyl guanidine whereby the copper sulfide is floated for recovery as a froth and the nickel sulfide is depressed.

WILLIAM KELVIN SPROULE.  
GEORGE ALAN HARCOURT.  
ERNEST HERBERT ROSE.

#### REFERENCES CITED

The following references are of record in the file of this patent:

Engineering and Mining Journal, Nov. 10, 1930, pages 466-472.

Milling Methods, 1930, pages 313 to 320, and 341.

#### Certificate of Correction

Patent No. 2,432,456.

December 9, 1947.

WILLIAM KELVIN SPROULE ET AL.

It is hereby certified that errors appear in the printed specification of the above numbered patent requiring correction as follows: Column 3, line 20, insert a comma after the word "converter"; column 4, line 31, Example No. 1, right hand column, under the heading "Per cent", for "23" read .23; column 5, line 53, for "370 F." read 370° F.; column 6, line 34, for "ean" read can; column 8, line 31, claim 7, for "0 25" read 0.25; lines 32 and 33, same claim, for "mass", each occurrence, read matte; line 57, claim 9, for "0 25" read 0.25; and that the said Letters Patent should be read with these corrections therein that the same may conform to the record of the case in the Patent Office.

Signed and sealed this 13th day of April, A. D. 1948.

[SNAL]

THOMAS F. MURPHY,  
Assistant Commissioner of Patents.

mass to froth flotation while maintaining a pH of about 10.0 to about 12.4 whereby the copper sulfide is floated as a copper concentrate and the nickel sulfide is depressed as a nickel concentrate, and further purifying the copper concentrate by successive froth flotation steps in the presence of diphenyl guanidine.

11. A process for recovering copper sulfide and nickel sulfide from bessemer matte which comprises slowly cooling said bessemer matte from the molten state to a temperature below about 950° F., comminuting the slowly-cooled matte in the presence of a sufficient quantity of an alkaline reagent to maintain a pH of about 10.0 to about 12.4, adding about 0.25 to about 1.0 pound of a compound selected from the group consisting of diphenyl guanidine and diortho tolyl guanidine per ton of matte, and subjecting the comminuted mass to froth flotation whereby copper sulfide is floated and recovered in the froth as a copper concentrate, the nickel sulfide being depressed as a nickel concentrate.

12. A process for separating nickel sulfide from copper sulfide which comprises subjecting a comminuted copper-nickel matte substantially devoid of iron and containing discrete particles of nickel sulfide and copper sulfide to selective froth flotation after adding about 0.25 to about 1.00 pound of a compound selected from the group consisting of diphenyl guanidine and diortho tolyl guanidine per ton of matte while maintaining a pH of about 10.0 to about 12.4 whereby the copper sulfide is floated for recovery in the froth and the nickel sulfide is depressed.

13. A process for separating nickel sulfide from copper sulfide which comprises subjecting a comminuted smelted mass substantially devoid of iron and containing discrete particles of nickel sulfide and copper sulfide to selective froth flotation after adding a compound selected from the group consisting of diphenyl guanidine and diortho tolyl guanidine while maintaining a pH of about 10 to about 12.4 and a pulp density between about 10% and about 40% solids whereby the copper sulfide is floated for recovery in the froth and the nickel sulfide is depressed.

14. A process for separating and recovering nickel sulfide and copper sulfide as concentrates from a bessemer matte containing mechanically joined crystals of nickel sulfide and copper sulfide which comprises comminuting said matte in a saturated aqueous solution of hydrated lime, adding about 0.25 to about 1.00 pound of diphenyl guanidine per ton of matte while grinding, subjecting the comminuted matte to froth flotation whereby the copper sulfide is floated as a copper concentrate and the nickel sulfide is depressed as a nickel concentrate, further purifying the copper concentrate by successive froth flotation steps in the presence of diphenyl guanidine, and combining the nickel concentrates from said froth flotation steps.

15. A process for separating nickel sulfide from copper sulfide which comprises subjecting a comminuted smelted mass substantially devoid of iron and containing discrete particles of nickel sulfide and copper sulfide to selective froth flotation while maintaining a pH of about 10 to about 12.4 after having added diphenyl guanidine whereby the copper sulfide is floated for recovery as a froth and the nickel sulfide is depressed.

16. A process for separating nickel sulfide from copper sulfide which comprises subjecting a comminuted bessemer matte containing discrete particles of nickel sulfide and copper sulfide to selective froth flotation while maintaining a pH of about 10 to about 12.4 after adding a compound selected from the group consisting of diphenyl guanidine and diortho tolyl guanidine whereby the copper sulfide is floated for recovery as a froth and the nickel sulfide is depressed.

WILLIAM KELVIN SPROULE.  
GEORGE ALAN HARCOURT.  
ERNEST HERBERT ROSE.

#### REFERENCES CITED

The following references are of record in the file of this patent:

Engineering and Mining Journal, Nov. 10, 1930, pages 466-472.

Milling Methods, 1930, pages 313 to 320, and 341.

#### Certificate of Correction

Patent No. 2,432,456.

December 9, 1947.

WILLIAM KELVIN SPROULE ET AL.

It is hereby certified that errors appear in the printed specification of the above numbered patent requiring correction as follows: Column 3, line 20, insert a comma after the word "converter"; column 4, line 31, Example No. 1, right hand column, under the heading "Per cent", for "23" read .23; column 5, line 53, for "370 F." read 370° F.; column 6, line 34, for "ean" read can; column 8, line 31, claim 7, for "0 25" read 0.25; lines 32 and 33, same claim, for "mass", each occurrence, read matte; line 57, claim 9, for "0 25" read 0.25; and that the said Letters Patent should be read with these corrections therein that the same may conform to the record of the case in the Patent Office.

Signed and sealed this 13th day of April, A. D. 1948.

[SNAL]

THOMAS F. MURPHY,  
Assistant Commissioner of Patents.